# EUROPEAN PATENT SPECIFICATION

(11) **EP 0 175 200 B1**
(45) Date of publication and mention of the grant of the patent: **27.06.1990**
(21) Application number: 85111031.2
(22) Date of filing: 02.09.1985
(51) Int. Cl.: D01F 9/14

(54) **Process for producing a carbon fiber from pitch material**
Verfahren zur Herstellung einer Kohlenstoffaser aus Pechmaterial
Procédé pour fabriquer une fibre de carbone à partir d'un brai

(30) Priority: 11.09.1984 JP 190404/84
(43) Date of publication of application: 26.03.1986
(73) Proprietor: MITSUBISHI KASEI CORPORATION, Tokyo 100 (JP)
(72) Inventor: Kagizaki, Masami, Kitakyushi-shi Fukuoka-ken (JP); Takakura, Tsuyoshi, Kitakyushi-shi Fukuoka-ken (JP); Tahara, Hiroshi, Kitakyushu-shi Fukuoka-ken (JP)
(74) Representative: Wächtershäuser, Günter, Prof. Dr.

(56) References cited:
- EP-A- 0 133 457
- EP-A- 0 149 348
- FR-A- 2 071 948
- US-A- 4 009 248

## Description

The present invention relates to a process for producing a carbon fiber from pitch material such as a coal-originated pitch, a petroleum pitch or a baked polymer pitch. More particularly, it relates to a process for producing such a pitch-type carbon fiber of high quality which is composed of carbon fiber monofilaments bound together without direct adhesion or fusion to one another, and which is easy to handle.

Pitch-type carbon fibers are produced usually by melt-spinning the pitch material to form precursory pitch fibers and subjecting the precursory pitch fibers to infusible treatment and carbonization treatment. Such pitch-type carbon fibers have an advantage that they can be produced in good yield and at low costs as compared with carbon fibers made of e.g. polyacrylonitriles. On the other hand, they have a disadvantage that the precursory pitch fibers are extremely brittle and difficult to handle for the infusible treatment or carbonization treatment. The precursory pitch fibers are likely to undergo fluffing, twine round guide rollers or break during such treatments. Further, there are additional difficulties such that adhesion or fusion is likely to take place among the precursory pitch fibers during the infusible treatment and the carbonization treatment, and the resulting carbon fiber surface is susceptible to damages.

These problems are substantially different from the problems involved in the case of the polyacrylonitrile-type carbon fiber which differs from the pitch-type carbon fiber in the starting materials as well as in the manner of the production. Namely, in the case of the polyacrylonitrile-type carbon fiber, a molten polyacrylonitrile is subjected to wet spinning in which it is extruded through spinning nozzles into a spinning bath composed essentially of a mixture of dimethylformamide with water or a mixture of dimethylsulfoxide with water and thereby forms solidified fibers. In such a wet spinning method, the; formed fibers are wetted with the solution of the spinning bath and bundles into a tow in the spinning bath. The tow withdrawn from the spinning bath is subjected to flame resistant treatment in an oxidizing atmosphere at a temperature of from 200 to 300°C and then to carbonization treatment in an inert atmosphere at a temperature of from 300 to 1400°C. For such treatments, it is considered effective to apply a lubricant such as polyethylene glycol or polypropylene glycol to the surface of the tow. However, when such a lubricant is used as an oiling agent for the step of bundling precursory pitch fibers, there will be difficulties such that the precursory pitch fibers are thereby partly dissolved, or the fibers tend to adhere or fuse to one another, whereby the tow tends to be stiff or rigid.

In US-A-4.009,248 it has been proposed to use as the starting material an acrylonitrile fiber which has been made to contain a particular aminosiloxane in the fiber production step for increasing operation efficiency and producing the carbon fiber in an extremely short firing time.

As a method for overcoming the difficulties in the bundling of the precursory pitch fibers, the present inventors have previously proposed to use a silicone oil as the oiling agent for bundling (EP-A-0 133 457) (not prepublished).

According to this method, the bundling can smoothly be conducted. However, depending upon the operation, the silicone oil may be applied excessively. While not adversely affecting the bundling operation, such excessive application of silicone oil is likely to lead to difficulties such that the tow of precursory pitch fibers tends to be stiff after the infusible treatment or the carbonization treatment, and in an extreme case, the pitch fibers tend to fuse one another to form a tow which is hardly unbound or separated into individual fibers.

Under these circumstances, the present inventors have conducted further researches to overcome these difficulties. As a result, they have found it effective to use an aqueous emulsion of a silicone oil as the oiling agent. The present invention has been accomplished based on this discovery.

Namely, the present invention provides a process for producing a carbon fiber from pitch material, which comprises melt spinning pitch material in a gaseous atmosphere to form precursory pitch fibers and bundling the precursory pitch fibers, followed by infusible treatment and carbonization and optionally by graphitization, characterized in that an aqueous emulsion of a silicone oil is applied as an oiling agent to the precursory pitch fibers prior to or during the bundling operation.

Now, the present invention will be described in detail with reference to the preferred embodiments.

As the pitch material to be used in the present invention, there may be mentioned a coal-originated pitch such as coal tar pitch or liquefied coal; a petroleum pitch such as a distillation residue obtained by the distillation of crude oil under atmospheric or reduced pressure or a heat-treated product thereof, or a heat-treated product of by-product tar obtained by the pyrolysis of naphtha; and a baked polymer pitch obtained by the carbonization of a synthetic or natural resin.

The melt spinning of the pitch material is conducted by extruding it into a gaseous atmosphere through spinning nozzles in the same manner as in the case of the dry melt spinning of ordinary synthetic fibers. It is preferred to employ a method wherein the pitch material is melted by an extruder or the like and extruded into a gaseous atmosphere from spinning nozzles directed downwardly, whereupon the extruded fibers are cooled and solidified. It is usual to employ spinning nozzles with discharge outlets havinag a diameter of from 0.1 to 0.5 mm. The temperature of the spinning nozzles is determined depending upon the type of the pitch material to provide a melt viscosity most suitable for spinning, and it is usually selected within a range of from 250 to 350°C. It is effective for the stabilization of spinning to provide temperature- keeping cylinders below the spinning nozzles.

In the present invention, an aqueous emulsion of a silicone oil is applied as an oiling agent to the precursory pitch fibers obtained by the spinning, prior to or during the bundling operation. As a specific example of such a silicone oil, dimethylpolysiloxane is usually employed. It is also possible to employ modified dimethylpolysiloxane derivatives obtained by introducing various groups to dimethylpolysiloxane. Specifically, there may be mentioned, for example, methylphenylpolysiloxane or hydrodiene- polysiloxane. Further, there may be employed other derivatives obtained by modifying dimethylpolysiloxane with one or more groups selected from the group consisting of an epoxy group, an alkyl group such as ethyl or propyl, an amino group, a carboxyl group, an alcohol, a phenyl group or a polyether. These silicone oils may be used alone or in combination as a mixture of at least two different kinds.

The aqueous emulsion of a silicone oil may be prepared by mixing the silicone oil with water by means of a common mixing device such as a high speed mixer, a colloid mill or a homogenizer so that the silicone oil constitutes from 0.1 to 35% by weight in the mixture. For the preparation of the emulsion, if the concentration of the silicone oil is too high to maintain the emulsified condition, from 0.25 to 2% by weight of an emulsifier may be added. As such an emulsifier, there may be employed conventional emulsifiers. For instance, there may be mentioned a nonionic emulsifier such as a sorbitan fatty acid ester e.g. sorbitan palmitic acid ester, sorbitan stearic acid ester, polyoxyethylene sorbitan fatty acid ester or polyoxyethylene sorbitan caproic acid ester, polyoxyethylene lauric acid ester, acetylated monoglyceride, acetylated glyceryl monostearate or a polyoxyethylene lanolin derivative; an anionic emulsifier such as an alkyl sulfate, sodium laurylsulfate, sodium cetylsulfate, a dialkyl sulfosuccinate or sodium di-2-ethylhexyl sulfosuccinate; or a cationic emulsifier such as alkyl pyridinium chloride. Further, a small amount of fine solid particles may be added to the aqueous emulsion of a silicone oil.

As the fine solid,partides, there may be employed, for instance, fine carbonaceous particles, fine inorganic oxide particles, fine inorganic salt particles or a mixture thereof. Specifically, there may be mentioned fine particles of graphite, carbon black, silica, calcium carbonate, titanium oxide, talc, clay, barium sulfate, potassium titanate or molybdenum disulfide.

The oiling agent may be applied to the precursory pitch fibers by various methods such as a spraying method, a roller coating method or a dipping method.

The amount of the deposition of the oiling agent onto the fibers is usually from 1 to 15% by weight, preferably from 2 to 10% by weight. If the amount of the deposition is less than 1 % by weight, it is difficult to maintain the bundled state of the spun fibers adequately, whereby it becomes difficult to handle the bundled fibers, and the fibers are likely to be damaged. On the other hand, if the amount exceeds 15% by weight, depending upon the concentration of the oiling agent, the evaporation at the time of the infusible treatment will be inadequate, and the agent will remain on the filaments and thus hinders the infusible reaction, and a low molecular weight gas genertated from the fibers during the infusible treatment will not sufficiently be dissipated, whereby the strength of the carbon fiber will be reduced.

The precursory pitch fibers having the aqueous solution of a silicone oil applied thereon and bundled, are subjected to infusible treatment and carbonization treatment in accordance with known methods. For instance, the infusible treatment may be conducted by heating the tow of fibers at a temperature of from 150 to 360°C for from 5 minutes to 10 hours in an oxidizing atmosphere such as oxygen, ozone, air, a nitrogen oxide, halogen or sulfur dioxide. The carbonization treatment may be conducted by heating the tow of fibers at a temperature of from 1000 to 2500°C for from 0.5 minute to 10 hours in an inert gas atmosphere such as nitrogen or argon.

Further, the graphitization may be conducted by heating the tow of fibers at a temperature of from 2500 to 3500°C for from 1 second to 1 hour.

If necessary, a load or tension may be applied to the tow of fibers to some extent during the infusible treatment, the carbonization treatment or the graphitization treatment for the purpose of preventing shrinkage or deformation.

Further, for the infusible treatment, it is desirable to preliminarily adjust the deposition of water on the precursory pitch fibers to a level of at most 0.1 % by weight either by providing a drier immediately before the infusible treatment furnace, or by drying, at the initial stage of the infusible treatment, the precursory pitch fibers at from 50 to 100°C for 5 minutes to 2 hours.

From the foregoing description, it should be understood that according to the present invention, the handling of brittle fibers can be made easy and it is possible to prevent the adhesion or fusion of the fibers to one another or to prevent the damages to the fiber surface, by a simple operation of applying an aqueous emulsion of a silicone oil to the precusory pitch fibers. Thus, a pitch-type carbon fiber having good quality is obtainable in the form of a continuous fiber in an industrially advantageous manner and condition. Further, the heat-treatments can thereby be conducted under uniform and sufficient tension, whereby a pitch-type carbon fiber having superior properties is obtainable at low costs.

Now, the present invention will be described in further detail with reference to Examples.

### Examples 1 to 4

Coal tar-originated pitch material (meso-phase pitch having an optical anisotropy of 100%) was melt- spun into a gaseous atmosphere at a spinneret temperature of 330°C. Then, an oiling agent as identified in Table 1 was applied by spraying to the precursory pitch fibers having a diameter of 10 pm thereby obtained, and the fibers were bundled together. The bundled fiber (i.e. tow) was dried in air at 80°C for 30 minutes. Then, it was heated from 150°C to 350°C over a period of 2 hours 40 mintues and held at that temperature for 30 minutes to conduct infusible treatment. Then, the fiber was subjected to carbonization treatment by heating it in argon from room temperature to 1,400°C over a period of 2 hours 20 minutes, and then maintaining it at that temperature for one hour, whereby a carbon fiber was obtained. The state of the bundling of fibers, the state of the fibers after the infusible treatment and the adhesion or fusion of monofilaments during the process of the production of the carbon fiber, were observed, and the tensile strength of the carbon fiber was measured. The results are shown in Table 1.

### Comparative Examples 1 to 5

The operation was conducted in the same manner as in Example 1 except that no oiling agent was used or the amount or the type of the oiling agent was varied. The results are shown in Table 1.

## Claims

1. A process for producing a carbon fiber from pitch material, which comprises melt spinning pitch material in a gaseous atmosphere to form precusory pitch fibers and bundling the precursory pitch fibers, followed by infusible treatment and carbonization and optionally by graphitization, characterized in that an aqueous emulsion of a silicone oil is applied as an oiling agent to the precursory pitch fibers prior to or during the bundling operation.

2. The process according to Claim 1, wherein the concentration of the silicone oil in the oiling agent is from 0.1 to 35% by weight.

3. The process according to Claim 1, wherein the oiling agent is applied in an amount of from 1 to 15% by weight relative to the fibers.

## Patentansprüche

1. Verfahren zur Herstellung einer Kohlenstofffaser aus Pechmaterial, umfassend das Schmelzspinnen von Pechmaterial in einer gasförmigen Atmosphäre zur Bilding von Vorläuferpechfasern und Bündelung der Vorläuferpechfasern, gefolgt von Unschmelzbar-Behandlung und Carbonisierung und gegebenenfalls von Graphitisierung, dadurch gekennzeichnet, daß man vor oder während der Bündelungsoperation eine wässrige Emulsion eines Siliconöls als ein Ölungsmittel auf die Vorläuferpechfasern appliziert.

2. Verfahren gemäß Anspruch 1, wobei die Konzentration des Siliconöls in dem Ölungsmittel von 0,1 bis 35 Gew.-% beträgt.

3. Verfahren gemäß Anspruch 1, wobei das Ölungsmittel in einer Menge von 1 bis 15 Gew.-%, bezogen ; auf die Fasern, appliziert wird.

## Revendications

1. Procédé de fabrication de fibres de carbone à partir d'une matière du type brai, qui comprend le filetage à l'etat fondu de la matière du type brai, dans une atmosphère gazeuse, pour former des fibres de brai précurseurs, et la mise sous forme de faisceaux des fibres de brai précurseurs, en faisant suivre par un traitement destiné à rendre ces dernières infusibles et une carbonisation et, facultativement, une graphitisation, caractérisé par le fait qu'on applique une émulsion aqueuse d'une huile de silicone, en tant qu'agent de lubrification, sur les fibres de brai précurseurs, avant ou pendant l'opération de mise sous forme de faisceaux.

2. Procédé selon la revendication 1, dans lequel la concentration de l'huile de silicone dans l'agent de lubrification va de 0,1 à 35% en poids.

3. Procédé selon la revendication 1, suivant lequel on applique l'agent de lubrification en une quantité allant de 1 à 15% en poids par rapport aux fibres.
